

- [54] **CELLULOSE ACETATE FIBER TOBACCO SMOKE FILTER AND PROCESS OF MANUFACTURING THE SAME**

[75] Inventors: **Masakazu Honda; Atsushi Saito; Sota Miyazawa; Keiji Kawabe, all of Toyama, Japan**

[73] Assignee: **Mitsubishi Acetate Company Limited, Tokyo, Japan**

[22] Filed: **Dec. 17, 1971**

[21] Appl. No.: **209,434**

[30] Foreign Application Priority Data

Dec. 18, 1970 Japan..... 45/113215

- |      |                      |                  |
|------|----------------------|------------------|
| [52] | U.S. Cl.....         | 131/267, 131/269 |
| [51] | Int. Cl.....         | A24b 15/02       |
| [58] | Field of Search..... | 131/261, 269     |

**[56] References Cited**

UNITED STATES PATENTS

- |           |         |                    |         |
|-----------|---------|--------------------|---------|
| 3,620,227 | 11/1971 | Saito et al. ....  | 131/269 |
| 3,477,445 | 11/1969 | Price et al. ....  | 131/267 |
| 3,443,566 | 5/1969  | Yasuda et al. .... | 131/267 |

#### OTHER PUBLICATIONS

Organic Chemistry (Text) by Fieser and Fieser Third Edition pub. by The Reinhold Publishing Corp. New

York 1956, pages 412,413 and 414 cited.

*Primary Examiner*—Melvin D. Rein  
*Attorney*—James E. Armstrong et al.

[57] ABSTRACT

A tobacco smoke filter effective for removing harmful and irritating substances from the tobacco smoke comprises a rod-like cellulose acetate fiber mass and a lubricant applied to the fiber mass and comprising a polyalkylene glycol-fatty acid-succharose ester ether of the formula:



wherein one of  $R_1$  to  $R_8$  is a polyalkylene glycol ether residue, at least one other is an acyl group having two to 19 carbon atoms and all the remainder are a hydrogen atom, and a polyglycerol-fatty acid ester in which the polyglycerol group has a degree of polymerization of two to three and the fatty acid has 12 to 22 carbon atoms, and, if desired, an edible mineral oil.

**10 Claims, No Drawings**

**CELLULOSE ACETATE FIBER TOBACCO SMOKE  
FILTER AND PROCESS OF MANUFACTURING  
THE SAME**

The present invention relates to a tobacco smoke filter and a process of manufacturing the same, more particularly, relates to a cellulose acetate fiber tobacco smoke filter containing a lubricant effective for removing substances harmful and irritating to health from the tobacco smoke and for enriching flavor and mildness of the tobacco smoke and a process of manufacturing the same.

In order to remove the harmful and irritating substances from the tobacco smoke, it is effective to filter the tobacco smoke through a filter composed of cellulose acetate fibers, filter paper, activated carbon, silica gel, polyethylene glycol or a composition of two or more of the above materials. Especially, it is well-known that the cellulose acetate fiber is a very effective material for removing nicotine, tar and other substances harmful and irritating to health. Accordingly, the cellulose acetate fiber is generally utilized for manufacturing a tobacco smoke filter.

In the manufacture of the tobacco smoke filter, it is necessary that the filter fibers have the following properties;

- (1) high processability in the formation of filter tip from filament tow,
- (2) high stability of filter form,
- (3) high property of removed of harmful and irritating substance from the tobacco smoke, and
- (4) a property of highly enriching the flavor and mildness of the tobacco smoke.

The tobacco smoke filter made of the filter fibers is required to have a pertinent smoke permeability and a high filtering efficiency to harmful and irritating substances such as tar, nicotine and other alkaloids.

Generally, the cellulose acetate filament tow usable for producing the tobacco smoke filter tips is prepared in a process wherein cellulose acetate flakes are dissolved into an organic solvent such as acetone, methylene chloride, and methanol, the solution is subjected to dry-spinning process, and then spun filaments are associated into a filament tow.

The filament tow thus produced is subjected to subsequent processing steps. In order to enhance the processability of the filament tow, the filament tow is generally impregnated with an aqueous emulsion containing a lubricant mainly consisting of mineral oil emulsified by a neutral surface active agent.

Therefore, the lubricant is required to impart to the filament tow a high processability and stability in continuous drawing, winding and other steps, a high uniformity of crimp on the filament tow without skip which means non-crimped portions of about 3/16 inch to about 12/16 inch in length in the crimped filament, and a high opening property when the filament tow is opened to a filament web. Further, it is desired that the lubricant enhance the effect of the filter tip on removal of nicotine, tar or other harmful and irritating substances, and increase the rigidity of the filter tip without increasing the resistance to smoke flow through the filter tip. Still further, it is preferable that the lubricant impart to the cigarette smoke an enriched flavor and mildness.

It is known that fatty acid saccharose ester is applied as a lubricant to the filament tow for tobacco smoke filter. However, it is difficult to apply the fatty acid saccharose ester lubricant to the filament tow uniformly due to low stability of the aqueous emulsion containing it.

That is, the low stability of the lubricant aqueous emulsion results in separation of the lubricant from the aqueous emulsion, so that the concentration of the lubricant in the aqueous emulsion changes with time and the separated lubricant deposits on the periphery of the roller disposed in the lubricant bath and carrying the aqueous emulsion to the filament tow.

Such non-uniform lubrication of the filament tow results in a number of disadvantages such as uneven crimps on the filament tow, high frictional resistance of the filaments to each other and to the processing device for example, the filament tow guide members, rollers and others, frequent breakages of the filament, and formation of numerous fibrils on the filament tows.

These disadvantages result in further uneven entanglements of the filaments in the tow and still further result in an uneven filament web when the filament tow is opened.

When the tobacco smoke filter tip is made from an unevenly lubricated filament tow as above, there results frequent generation of electro-static charges on the filaments. The electro-static charge causes difficulty in rolling up of the filament web into a rod so that the rolling up operation is frequently stopped and the rolling up machine must be subjected to frequent regulation and cleaning thereof. Further, the tobacco smoke filters from the unevenly lubricated filament tow result in non-uniformity of the flavor and mildness of the tobacco smoke.

The inventors have searched for a long time for a neutral surface active agent effective for uniformly emulsifying the fatty acid saccharose ester and, if necessary, mineral oil into water without obstructing the beneficial properties of the fatty acid saccharose ester such as the ability to remove harmful and irritating substances from the tobacco smoke and the property of enriching the flavor and mildness of tobacco smoke.

From the study, it has been found that polyglycerine fatty acid ester is a neutral surface active agent suitable for use as the lubricant for the cellulose acetate filament tow.

One of objects of the present invention is to provide a cellulose acetate fiber tobacco smoke filter effective for removing harmful and irritating substances from tobacco smoke and a process of manufacturing the same.

Another object of the present invention is to provide a cellulose acetate fiber tobacco smoke filter effective for imparting enriched flavor and mildness to tobacco smoke and a process of manufacturing the same.

A further object of the present invention is to provide a cellulose acetate fiber tobacco smoke filter having a pertinent rigidity and resistivity against smoke flow and a process of manufacturing the same.

The tobacco smoke filter of the present invention comprises a short-length, rod-like cellulose acetate fiber mass and a lubricant applied to the cellulose acetate fiber mass and containing five to 35 parts by weight of a polyalkylene glycol-fatty acid saccharose ester ether of the formula:



wherein one of  $R_1$ ,  $R_2$ ,  $R_3$ ,  $R_4$ ,  $R_5$ ,  $R_6$ ,  $R_7$  and  $R_8$  represents a monovalent polyalkylene glycol ether residue, at least one other represents a monovalent acyl group having two to 19 carbon atoms and all the remainder represent a hydrogen atom, and five to 65 parts by weight of an ester of a fatty acid having 12 to 22 carbon atoms with a polyglycerin having a degree of polymerization of two to three.

The cellulose acetate fiber tobacco smoke filter of the present invention is manufactured by impregnating a cellulose acetate filament tow with an aqueous emulsion of a lubricant as mentioned above, crimping the filament tow, forming the crimped filament tow into tobacco smoke filter rod and cutting the rod into tips.

The fatty acid saccharose ester usable for the present invention is an ester ether of disaccharide having one polyalkylene glycol ether residue and one or more fatty acid ester residue, that is, a member of an acyl group, more concretely, in an ester ether of pyranose and furanose type disaccharide represented by the formula:



wherein one of  $R_1$ ,  $R_2$ ,  $R_3$ ,  $R_4$ ,  $R_5$ ,  $R_6$ ,  $R_7$ ,  $R_8$  is a monovalent polyalkylene glycol ether residue, at least one other of them is a monovalent fatty acid ester residue having two to 19 carbon atoms and all the remainder are a hydrogen atom.

In the saccharide ester ether, the fatty acid ester residue, namely, the acyl group may be selected from the group consisting of acid residues of lauric acid, coconut fatty acid, palmitic acid, stearic acid, oleic acid, or beef tallow fatty acid, and the polyalkylene glycol ether residue may be an ether residue of polyethylene glycol, polypropylene glycol, polyethylene-propylene glycol, polybutylene glycol and other polyalkylene glycol in which five to 30 mols of glycol units are polymerized.

The polyglycerine fatty acid ester usable for the present invention is prepared by the ester reaction of a fatty acid, for example, lauric acid, coconut fatty acid, palmitic acid, stearic acid, oleic acid and beef tallow fatty acid with a polyglycerine having a degree of polymerization of two to three which is obtained by heat-polycondensation of glycerine at a high temperature.

The lubricant usable for the present invention contains five to 35 parts by weight of the polyalkylene glycol fatty acid saccharose ester ether and five to 65 parts by weight of polyglycerine fatty acid ester, and if desired, a mineral oil usable as a food additive or medical additive. It is necessary that the edible mineral oil meets the Japanese Pharmacopoeia Standard Requirements as to phase, pH, contents of solid paraffins and sulfur compounds, nitronaphthalene test and sulfur color test and meets the U. S. Food Additive Standard Requirements as to the ultraviolet rays absorption test.

The lubricant usable for the present invention may contain certain neutral surface active agents other than the polyglycerine fatty acid ester and usable as a food additive and medical additive.

- 5 The lubricant is emulsified into water preferably in a concentration of 0.5 to 10 percent by weight and applied to the cellulose acetate filament tow so as to leave 0.5 to 5.0 percent of the lubricant based on the weight of the filament tow, on the filament tow.
- 10 The cellulose acetate filament tow thus lubricated is valuable for producing a tobacco smoke filter in a favourable condition and for obtaining tobacco smoke filter tips having high benefits in chemical and physical properties, that is, the removal of harmful and irritating substances from tobacco smoke and the enrichment of flavour and mildness of tobacco smoke.

In the manufacture of the tobacco smoke filter of the present invention, a cellulose acetate filament tow is impregnated with an aqueous emulsion containing a lubricant as stated hereinbefore so as to apply a desired amount of the lubricant to the filament tow, the impregnated filament tow is crimped at a desired crimp number by a crimper and then the crimped filament tow is formed into filter rod. In the formation of the filter rod, the crimped filament tow is conditioned to a desired moisture content, and opened into a filament web and rolled up with paper into a rod form using a filter plug making machine. The rod is cut into filter plugs and thereafter, further cut into filter tips of desired length.

The following specific examples will more particularly illustrate the present invention.

#### Example 1

- 35 A lubricant aqueous emulsion was prepared by emulsifying 3 percent by weight of a lubricant consisting of 25 parts by weight of polyoxyethylene palmitic acid saccharose ester ether wherein the polyoxyethylene group consisted of 20 mols of ethylene oxide, 15 parts by weight of polyglycerol laurate wherein the polyglycerol group had a degree of polymerization of three and 60 parts by weight of an edible mineral oil satisfying the Japanese Pharmacopoeia Standard and the U. S. Food Additive Standard and had an SSU viscosity of 120 at a temperature of 37.8° C, into 97 percent by weight of water. The aqueous emulsion was charged into a lubrication bath having a rotatable roller lower half part of which was immersed in the aqueous emulsion.
- 40 A cellulose acetate filament tow having a Y-shaped cross-sectional profile, a single filament denier of four and a total denier of 43,000 was impregnated with the aqueous emulsion by bringing the filament tow into contact with the rotatable roller periphery carrying the aqueous emulsion while continuously advancing it forwardly. By the above process, the lubricant was applied to the filament tow in a content of approximately of 0.8 percent based on the weight of the filament tow.
- 45 The filament tow thus impregnated was crimped by a crimper at a crimp number of approximately 18 crimps/25 mm, and the crimped filament tow was conditioned into a predetermined moisture content and thereafter, packed in a package box.
- 50 The filament tow was continuously drawn out from the package box and uniformly opened. Using a filter plug making machine, the open filament web was rolled up with paper to form a rod of 7.9 mm diameter and
- 55
- 60
- 65

then the rod was cut into filter plugs of 102 mm length. A filter plug was further cut to form it into filter tips of 17 mm length.

For comparison, three kinds of Comparison Examples A, B and C were prepared by the same procedure as above except that the lubricant contained no polyglycerol laurate (Comparison Example A), no polyoxyethylene palmitic acid saccharose ester ether (Comparison Example B) and no polyglycerol laurate and polyoxyethylene palmitic acid saccharose ester ether (Comparison Example C).

The filter tips from the present example and Comparison Examples A, B and C were attached to cigarette ends by adhesive paper so as to obtain samples for organoleptic test.

With respect to the present example and Comparison Examples A, B and C, the lubricant aqueous emulsions, the impregnated filament tows, the filter tips and the cigarette with a filter tip were subjected to measurement in the items as shown in Table 1.

Table 1 shows the results of the measurements.

The removal efficiency for alkaloid was determined according to ultraviolet rays absorption spectrum analysis.

The organoleptic test was carried out by 20 panel members with respect to the six items of flavor, taste, smell, mildness, general quality and others, and significant differences between the cigarettes for every item were recorded.

Referring to Table 1, it is clear that the lubricant of Example 1 gives a higher stability to the aqueous emulsion, a more uniform appearance and a higher opening property to the filament tow, a higher rigidity and removal efficiencies for tar and alkaloids to the filter tip and richer mildness to the cigarette than those of Comparison Examples A, B and C.

### Example 2

The procedure of Example 1 was repeated using an aqueous emulsion containing five percent by weight of a lubricant consisting of 20 parts by weight of polyoxy-

TABLE 1

| Material     | Item                                                   | Example 1             | Comparison example    |                         |                                            |
|--------------|--------------------------------------------------------|-----------------------|-----------------------|-------------------------|--------------------------------------------|
|              |                                                        |                       | A                     | B                       | C                                          |
| Emulsion     | Stability                                              | Excellent             | Good                  | Good                    | Unstable.                                  |
|              | Crimping property                                      | Good                  | do                    | do                      | Good.                                      |
| Filament Tow | Appearance of crimped tow.                             | Substantially no skip | Small number of skips | Substantially no skip   | Small number of skips.                     |
|              | Opening property                                       | Excellent             | Good                  | Good                    | Good.                                      |
|              | Weight (g.)                                            | 0.12                  | 0.12                  | 0.12                    | 0.12                                       |
|              | Rigidity (1/10 mm.)                                    | 8.2                   | 8.4                   | 8.5                     | 8.6                                        |
|              | Resistivity against ventilation (mm. H <sub>2</sub> O) | 46                    | 44                    | 45                      | 44                                         |
| Filter tip   | Removal efficiency for tar (percent)                   | 39.2                  | 39.0                  | 38.5                    | 38.2                                       |
|              | Removal efficiency for alkaloids (percent)             | 33.8                  | 29.4                  | 32.1                    | 30.7                                       |
| Cigarette    | Organoleptic test                                      | Rich mildness         | Good                  | Somewhat poor mildness. | Poor mildness and a slight oil-like smell. |

Measuring methods for the items shown in Table 1 were as follows.

The stability of the lubricant aqueous emulsion was determined by standing 3, 5 and 10 percent lubricant aqueous emulsions at a temperatures of 20°, 30° and 40° C for 10 days and observing changes during the standing, and observed significant differences between the emulsions were recorded.

The crimping property of the filament tow and the appearance of the crimped filament tow were determined according to the method of JIS L-1036, and significant differences between the filament tows were recorded.

The opening property of the filament tow was determined using a Sleddit Roll type opening device, and significant differences between the filament tows were recorded.

The weight of the filter tips of 17 mm length was measured.

The rigidity was expressed by the depth (in 1/10 mm) of a recess formed on the periphery of the filter tip of 17 mm length by pressing against it with a circle plate of 12 mm diameter under a load of 300 g.

The resistivity against ventilation was expressed by the pressure drop in mm H<sub>2</sub>O when the air was flowed through the filter tip of 17 mm length at a flow rate of 17.5 ml/sec.

The removal efficiency for tar was determined by having a cigarette with a filter tip of 17 mm length smoked by an automatic smoking device and measuring the weights of the filter tip before and after smoking.

ethylene palmitic acid sacharose ester ether in which the polyoxyethylene group consisted of 20 moles of ethylene oxide, 15 parts by weight of polyglycerol laurate in which the polyglycerol group had a degree of polymerization of three, 10 parts by weight of polyoxyethylene iso-stearate in which the polyoxyethylene group consisted of 15 mols of ethylene oxide and 55 parts by weight of an edible mineral oil which had an SSU viscosity of 120 at 37.8° C and satisfying the Japanese Pharmacopoeia Standard and the U. S. Food Additive Standard.

After the impregnating step, the cellulose acetate filament tow containing 1.0 percent of the lubricant based on the weight of the filament tow, was crimped at a crimp number of approximately 18 crimps/25 mm by a crimper. The crimped filament tow was conditioned into a predetermined moisture content and packed into a package box.

Filter tips similar to those of Example 1 were prepared from the filament tow thus packed in the package box.

For comparison, a filter tip (Comparison Example D) was prepared by the same procedure as above using as the lubricant the mixture of "Additional Item 12" of Japanese Pat. No. 319,066, consisting of 75 parts by weight of mineral oil and 25 parts by weight of a mixture of sorbitan monolaurate with polyoxyethylene sorbitan monolaurate in which the polyoxyethylene group consisted of 20 mols of ethylene oxide in equivalent mol number.

The filter tips of Example 2 and Comparison Example D were attached to cigarette ends by adhesive

paper in order to prepare testing specimens for an organoleptic test.

With respect to Example 2 and Comparison Example D, the lubricant aqueous emulsions, impregnated filament tows, filter tips and cigarettes with a filter tip were subjected to measurement in the items as shown in Table 2.

Table 2 shows all the results of the measurements.

ter tips of 12 mm length.

For comparison, the same procedure as above was repeated using a lubricant consisting only of the mineral oil same as above (Comparison Example E).

The filter tips of Example 3 and Comparison Example E were attached to cigarette ends by adhesive paper in order to prepare testing specimens for organoleptic test.

TABLE 2

| Material                                        | Item                                   | Example 2                     | Comparison Example D   |
|-------------------------------------------------|----------------------------------------|-------------------------------|------------------------|
| Emulsion                                        | Stability                              | Excellent                     | Good.                  |
| { Crimping property                             | Good                                   | Do.                           |                        |
| Filament tow                                    | Appearance of crimped tow              | Substantially no skip         | Substantially no skip. |
| { Opening property                              | Excellent                              | Good.                         |                        |
| { Weight (g.)                                   | 0.11                                   | 0.11.                         |                        |
| { Rigidity (1/10 mm.)                           | 8.3                                    | 8.5.                          |                        |
| { Resistivity against ventilation (mm. $H_2O$ ) | 29.7                                   | 29.2.                         |                        |
| Filter tip                                      | { Removal efficiency for tar (percent) | 26                            | 24.                    |
| { Removal efficiency for alkaloids (percent)    | 22                                     | 21.                           |                        |
| Cigarette                                       | Organoleptic test                      | Rich taste and good mildness. | Good.                  |

Referring to Table 2, it is evident that the lubricant of Example 2 is superior in the stability of the aqueous emulsion, opening property of the filament tow, rigidity, resistivity against ventilating and removing efficiencies for tar and alkaloids of the filter tip and taste and mildness of the cigarette more than those of Comparison Example D.

Table 3 shows properties of the filter tips and the cigarettes of Example 3 and Comparison Example E. From the table, it is clear that the filter tips and the cigarettes of Example 3 are superior in rigidity, resistivity against ventilation, removal efficiencies for tar and alkaloids and organoleptic properties to those of Comparison Example E.

TABLE 3

| Material                                        | Item              | Example 3 | Comparison Example E |
|-------------------------------------------------|-------------------|-----------|----------------------|
| Filter tip                                      | { Weight (g.)     | 0.11      | 0.11                 |
| { Rigidity (1/10 mm.)                           | 8.3               | 8.5       |                      |
| { Resistivity against ventilation (mm. $H_2O$ ) | 29.7              | 29.2      |                      |
| { Removal efficiency for tar (percent)          | 26                | 24        |                      |
| { Removal efficiency for alkaloids (percent)    | 22                | 19.5      |                      |
| Cigarette                                       | Organoleptic test | (1)       | (2)                  |

<sup>1</sup> Rich taste and good mildness.

<sup>2</sup> Poor mildness and a slight oil-like smell.

### Example 3

A cellulose acetate filament tow having regular cross-section, a single filament denier of 4 and a total denier of 55,000 was subjected to the same procedure as that of Example 1 using a 3 percent aqueous emulsion of a lubricant consisting of 20 parts by weight of polyoxyethylene lauric acid saccharose ester ether wherein the polyoxyethylene group consisted of 12 mols of ethylene oxide, 20 parts by weight of polyglycerol laurate wherein said polyglycerol group had a degree of polymerization of two and 60 parts by weight of an edible mineral oil having an SSU viscosity of 120 at a temperature of 37.8° C and satisfying the Japanese Pharmacopoeia Standard and the U. S. Food Additive Standard. The cellulose acetate filament tow contained 1.0 percent of the lubricant based on the weight of the filament tow, crimped at a crimp number of approximately 18 crimps/25 mm by a crimper, conditioned into a predetermined moisture content and then packed into a package box.

Thereafter, the filament tow was continuously drawn out from the package box and uniformly opened. Using a filter plug making machine, the open filament web was rolled up with paper to form a rod of 8.2 mm diameter, and the rod was cut into filter plugs of 72 mm length. The filter plug was further cut to form it into fil-

### Example 4

The same procedure as that of Example 1 was repeated using a 5 percent aqueous emulsion of a lubricant consisting of 20 parts by weight of polyoxyethylene lauric acid saccharose ester ether in which the polyoxyethylene group consisted of 12 mols of ethylene oxide, 20 parts by weight of polyglycerol laurate in which the polyglycerol group had a degree of polymerization of two, 15 parts by weight of polyglycerol oleate in which the polyglycerol group had a degree of polymerization of two, and 45 parts by weight of an edible mineral oil having an SSU viscosity of 120 at 37.8° C and satisfying the Japanese Pharmacopoeia Standard and the U. S. Food Additive Standard. The cellulose acetate filament tow contained 1.0 percent of the lubricant based on the weight of the filament tow.

The properties of the resultant filter tip and the cigarette are illustrated in Table 4 shown below.

### Example 5

The same procedure as that of Example 1 was repeated using a 5 percent aqueous emulsion of a lubricant consisting of 35 parts by weight of polyoxyethylene oleic acid saccharose ester ether in which the polyoxyethylene group consisted of 25 mols of ethylene oxide, 10 parts of polyglycerol oleate in which the poly-

glycerol group had a degree of polymerization of two and 55 parts by weight of an edible mineral oil satisfying the Japanese Pharmacopoeia Standard and the U. S. Food Additive Standard and having an SSU viscosity of 100 at 37.8° C. The cellulose acetate filament tow contained 1.3 percent of the lubricant based on the weight of the filament tow.

For comparison, the same procedure as above was repeated except that the lubricant consisted only of the mineral oil (Comparison Example F).

The resultant filter tips and the cigarettes of Example 5 and Comparison Example F had the properties as shown in Table 4 below.

#### Example 6

The same procedure as that of Example 1 was repeated using a 5 percent aqueous emulsion of a lubricant consisting of 20 parts by weight of polyoxyethylene oleic acid saccharose ester ether in which the polyoxyethylene group consisted of 25 mols of ethylene oxide, 60 parts of polyglycerol laurate wherein the polyglycerol group had a degree of polymerization of two and 20 parts by weight of an edible mineral oil satisfying the Japanese Pharmacopoeia Standard and the U. S. Food Additive Standard and having an SSU viscosity of 100 at 37.8° C. The cellulose acetate filament tow contained 1.0 percent of the lubricant based on the weight of the filament tow.

The properties of the resultant filter tip and the cigarette are shown in Table 4 below.

which the polyglycerol group had a degree of polymerization of two, 15 parts by weight of polyoxyethylene isostearate in which the polyoxyethylene consisted of 15 mols of ethylene oxide and 70 parts by weight of an edible mineral oil satisfying the Japanese Pharmacopoeia Standard and the U. S. Food Additive Standard and having an SSU viscosity of 120 at 37.8° C. The cellulose acetate filament tow contained 1.7 percent of the lubricant based on the weight of the filament tow.

10 The resultant filter tip and cigarette had the properties as shown in Table 4 below.

#### Example 9

15 The same procedure as that of Example 1 was repeated using a 10 percent aqueous emulsion of a lubricant consisting of 20 parts by weight of polypropylene glycol lauric acid saccharose ester ether in which the polypropylene glycol group had a molecular weight of approximately 400, 20 parts by weight of polyglycerol laurate in which the polyglycerol group had a degree of polymerization of two and 60 parts by weight of an edible mineral oil satisfying the Japanese Pharmacopoeia Standard and the U. S. Food Additive Standard and having an SSU viscosity of 120 at 37.8° C. The cellulose acetate filament tow contained 1.0 percent of the lubricant based on the weight of the filament tow.

25 The resultant filter tip and the cigarette had the properties as shown in Table 4 below.

TABLE 4

| Material   | Item                                                    | Example |      | Comparison |      | Example |      |      |
|------------|---------------------------------------------------------|---------|------|------------|------|---------|------|------|
|            |                                                         | 4       | 5    | F          | 6    | 7       | 8    | 9    |
| Filter tip | (Weight (g.).                                           | 0.12    | 0.11 | 0.11       | 0.11 | 0.13    | 0.11 | 0.11 |
|            | Rigidity (1/10 mm.).                                    | 8.4     | 8.5  | 8.6        | 8.5  | 8.3     | 8.3  | 8.4  |
|            | Resistivity against ventilation (mm. H <sub>2</sub> O). | 29.6    | 30.0 | 29.3       | 30.8 | 30.2    | 29.9 | 29.9 |
|            | Removal efficiency for tar (percent).                   | 25      | 26   | 24         | 26   | 27      | 26   | 25   |
|            | Removal efficiency for alkaloids (percent).             | 22      | 22   | 21         | 22   | 23      | 22   | 21   |
| Cigarette  | Organoleptic test.                                      | (1)     | (1)  | (2)        | (1)  | (3)     | (1)  | Good |

<sup>1</sup> Rich mildness.

<sup>2</sup> A little oil-like smell.

<sup>3</sup> Rich taste and good mildness.

#### Example 7

The same procedure as that of Example 1 was repeated using a 2.5 percent aqueous emulsion of a lubricant consisting of 30 parts by weight of polyoxyethylene palmitic acid saccharose ester ether in which the polyoxyethylene group consisted of 20 mols of ethylene oxide, 60 parts by weight of polyglycerol laurate in which the polyglycerol group had a degree of polymerization of two and 10 parts by weight of polyoxyethylene isostearate in which the polyoxyethylene group consisted of 15 mols of ethyleneoxide. The cellulose acetate filament tow contained 3.0 percent of the lubricant based on the weight of the fiber tow. The resultant filter tip and cigarette had the properties as shown in Table 4 below.

#### Example 8

The same procedure as that of Example 1 was repeated using a 10 percent aqueous emulsion of a lubricant consisting of five parts by weight of polyoxyethylene lauric acid saccharose ester ether in which the polyoxyethylene group consisted of 20 mols of ethylene oxide, 10 parts by weight of polyglycerol laurate in

#### What we claim is:

1. A cellulose acetate fiber tobacco smoke filter which comprises a rod-like cellulose acetate fiber mass and a lubricant applied to the fiber mass and containing five to 35 parts by weight of a polyalkylene glycol fatty acid saccharose ester ether having the formula:



60 whereon one of R<sub>1</sub>, R<sub>2</sub>, R<sub>3</sub>, R<sub>4</sub>, R<sub>5</sub>, R<sub>6</sub>, R<sub>7</sub> and R<sub>8</sub> represents a polyalkylene glycol ether residue, at least one other of them represents an acyl group having two to 19 carbon atoms and all the remainder represent a hydrogen atom, and five to 65 parts by weight of a polyglycerine fatty acid ester in which the polyglycerine residue has a degree of polymerization of two to three and the fatty acid residue has 12 to 22 carbon atoms.

2. A tobacco smoke filter as claimed in claim 1, wherein said lubricant further comprises 20 to 70 parts by weight of an edible mineral oil.

3. A tobacco smoke filter as claimed in claim 1, wherein the amount of said lubricant in said fiber bundle is 0.5 to 5.0 percent based on the weight of said fiber bundle.

4. A tobacco smoke filter as claimed in claim 2, wherein the amount of said lubricant in said fiber bundle is 0.5 to 5.0 percent based on the weight of said fiber bundle.

5. A tobacco smoke filter as claimed in claim 1, wherein said polyalkylene glycol ether residue is selected from the group consisting of the ether residues

of polyethylene glycol, polypropylene glycol, polyethylene-propylene glycol and poly-butylene glycol.

6. A tobacco smoke filter as claimed in claim 1, wherein said polyalkylene glycol ether residue consists of five to 30 moles of glycol units.

7. A tobacco smoke filter as claimed in claim 1, wherein said acyl group is selected from the group consisting of acid residues of lauric acid, palmitic acid stearic acid, oleic acid, coconut fatty acid and beef tallow fatty acid.

8. A tobacco smoke filter as claimed in claim 1, wherein the fatty acid residue of said polyglycerine fatty acid ester is selected from the group consisting of acid residues of lauric acid, palmitic acid, stearic acid, oleic acid, coconut fatty acid and beef tallow fatty acid.

15

20

25

30

9. A process of manufacturing a cellulose acetate fiber tobacco smoke filter which comprises impregnating a cellulose acetate filament tow with an aqueous emulsion of a lubricant containing 5 to 35 parts by weight of a polyalkylene glycol fatty acid saccharose ether ester having the formula:



wherein one of R<sub>1</sub>, R<sub>2</sub>, R<sub>3</sub>, R<sub>4</sub>, R<sub>5</sub>, R<sub>6</sub>, R<sub>7</sub> and R<sub>8</sub> represents a polyalkylene glycol ether residue, at least one other of them represents an acyl group having two to 19 carbon atoms and all the remainder represent a hydrogen atom, and five to 65 parts by weight of a polyglycerine fatty acid ester in which the polyglycerine residue has a degree of polymerization of two to three and the fatty acid residue has 12 to 22 carbon atoms, crimping said impregnated filament tow and forming said crimped filament tow into tobacco smoke filter rods.

10. A process as claimed in claim 9, wherein said lubricant further comprises 20 to 70 parts by weight of an edible mineral oil.

\* \* \* \* \*

35

40

45

50

55

60

65